

May 1, 1951

C. E. STEVENS, JR.

2,550,879

### BIMETALLIC PISTON

Filed Nov. 10, 1949

FIG. 1.



FIG. 2.

CHARLES E. STEVENS, JR. *INVENTOR.*

BY

Campbell, Brundage, Frost & Graves  
his ATTORNEYS.

## UNITED STATES PATENT OFFICE

2,550,879

## BIMETALLIC PISTON

Charles E. Stevens, Jr., Garden City, N. Y., assignor to Fairchild Engine and Airplane Corporation, Farmingdale, N. Y., a corporation of Maryland

Application November 10, 1949, Serial No. 126,627

10 Claims. (Cl. 309—14)

1

This invention relates to bimetallic articles and has particular reference to the insertion of a piston ring band into an aluminum piston.

It has been proposed heretofore to improve the wearing characteristics of aluminum pistons by inserting bands near the piston head in which the piston ring grooves are formed. Steel and cast iron have been suggested for such bands because of the improved wearing capacity of these metals over aluminum and aluminum base alloys. However, because of the widely different coefficients of thermal expansion between cast iron and steel on the one hand, and aluminum and aluminum base alloys on the other, it has been further proposed to incorporate in the iron and steel an alloying metal, such as nickel, which imparts thereto a coefficient of thermal expansion more nearly matching that of the aluminum or the aluminum base alloy constituting the body of the piston. However, even in that case, the disparity in thermal expansion between the inserted band and the aluminum base body of the piston causes the aluminum to "grow" against the restraining iron or steel band during the heating cycle, which results in minute upsetting of the aluminum so that when it cools, the band will not fit as tightly as it did originally. Subsequent heating cycles exaggerate this condition until the ring band finally becomes loose in the aluminum base piston and failure occurs. Therefore, while helpful and desirable, high nickel cast iron bands of high coefficient of expansion inserted in aluminum pistons do not entirely solve the problem.

In accordance with the present invention, aluminum base and aluminum base alloy pistons having wear reducing ring bands inserted therein are provided in which the ring band is molecularly bonded to the aluminum under such conditions that a difference in coefficient of thermal expansion between the aluminum and the ferrous metal is insufficient to produce a strain which will exceed the bond strength during cooling of the piston after the casting operation. Accordingly, the subsequent subjection of the piston to wide temperature fluctuations in operation will not result in rupture of the bond, and the ring band remains firmly seated in the piston, as has been demonstrated by rigorous testing in actual use.

2

In making the bimetallic piston of this invention, a ring band of high nickel cast iron of high coefficient of thermal expansion or a gray iron ring band of low modulus of elasticity is first coated with a thin film of molten aluminum overlying a ferro-aluminum alloy layer at the interface and, while the aluminum-coated ring band is at a temperature at least as high as the melting temperature at which the aluminum or 5 aluminum base alloy to be used as the body of the piston is cast and while the aluminum film on the band is molten or plastic, the aluminum body metal is cast around the ring band, preferably in a permanent mold according to known 10 casting techniques. When the piston is cooled and removed from the mold, the band will be 15 molecularly bonded to the aluminum through the intervening ferro-aluminum alloy layer, which is preferably held to a thickness on the 20 order of a thousandth of an inch because of its inherently brittle nature.

It will be seen that the bimetallic piston of this invention is a strong and wear-resistant composite product having the properties of lightness of 25 aluminum and strength of the cast iron or steel at the point where the greatest wear occurs and damage frequently results after short usage, and which is avoided by use of the piston of this invention.

For a more complete understanding of the invention, reference may be had to the accompanying drawing, in which:

Figure 1 is a cross-section through a bimetallic piston of this invention; and

Fig. 2 is an enlarged cross-section through the piston insert of Fig. 1 to illustrate the bimetallic arrangement in greater detail.

Referring to the drawing, numeral 10 designates a ring band of cast iron or cast steel inserted in a piston 11 of cast aluminum or aluminum base alloy. The ring band 10 preferably is formed as a complete ring, without the piston ring groove 12 which is machined therein after the composite iron-aluminum piston is formed. 40 Preferably also, the ring band 10 is larger in outside diameter than the piston, so that it may be properly located in a recess in the permanent mold into which the aluminum or aluminum base alloy is cast.

50 Prior to insertion in the mold, the cast iron

or steel ring band 10 is heated to the temperature at which aluminum alloys with the iron or steel, preferably by immersing the band 10 in a bath of molten aluminum or aluminum base alloy for a sufficient period of time to reach the said temperature, and then allowing the alloying action to take place between the surface metal of band 10 and the molten aluminum or aluminum base alloy, until the desirably thin layer of the alloy and the overlying aluminum film are formed thereon. Although the ferro-aluminum alloy is necessary to a molecular bond between the aluminum and ferrous metals constituting the composite piston, the brittleness of the alloy requires that the layer be kept down to a thickness on the order of a thousand of an inch.

The coated ring band 10, while heated to a temperature such that the surface film of aluminum is still molten or plastic, is then placed in the permanent mold of the desired configuration, and the molten aluminum or aluminum base alloy body metal 11 cast around the ring band 10. Owing to the fusion union between the molten or plastic film of aluminum on the ring band 10 and the molten casting metal, the aluminum is homogeneous outwardly from the surface of the ferro-aluminum alloy layer 13, which constitutes the molecular bond between the aluminum or aluminum alloy body 11 of the piston and the ferrous metal ring band 10. Further details of the general process for forming such bimetallic structures may be had upon reference to the Whitfield et al. Patent No. 2,396,730, issued March 19, 1946.

As is well known, the thermal and mechanical or impact and wear stresses to which the piston is subjected in use are of considerable magnitude, and therefore, minimization thereof is desirable in the first instance. Hence, the ring band 10 is desirably formed of a high nickel cast iron containing about 12.5% nickel, or more or less, in order to reduce the disparity in coefficients of thermal expansion between the material of which the ring band 10 is formed and the material of which the piston body 11 is formed. One suitable commercial form is marketed under the trade name "Ni-resist." This thermal expansion disparity may be further reduced by utilizing as material for the piston body 11, an aluminum base alloy containing alloying ingredients reducing the thermal expansion of aluminum. One such alloy is aluminum containing 12% silicon, 2.5% nickel, 1.2% magnesium and 0.8% copper, and is known commercially as Alcoa "Al32 alloy." Assuming that the aforementioned high nickel cast iron ring 10 and low expanding aluminum alloy body 11 are employed, an analysis of the stresses involved will show the conditions which enable the piston of this invention to withstand most rigorous usage without impairment beyond normal wear.

Assuming that insert 10 has an inside diameter at room temperature of 4.375 inches, its radial contraction ( $u$ ) from the solidification temperature of the Al32 alloy will be

$$u = 2.187'' \times 10.7 \times 10^{-6} \times (1085 - 70) = .024$$

The solidification temperature,  $\Delta T$ , as reflected by an identical shrinkage in Al32 alloy is

$$\begin{aligned} .024 &= 2.187 \times 12.3 \times 10^{-6} \times \Delta T \\ \Delta T &= \frac{.024}{2.187 \times 12.3 \times 10^{-6}} \\ &= 892^\circ \text{ F.} \end{aligned}$$

Adding a room temperature of  $70^\circ \text{ F.}$  brings the temperature up to  $962^\circ \text{ F.}$  This is an indication that the restraint offered by the cores in the mold give a casting having a final size which is the equivalent of a casting obtained with unrestrained cooling from a hypothetical solidification point of  $962^\circ \text{ F.}$  This indication is reasonable since it has been found that the restraint of a core is often more than this. To carry the analysis further, consider Alcoa 142 alloy containing 4% copper, 2.0% nickel and 1.5% magnesium, as substituted for the Al32 alloy, and using the  $\Delta T$  of  $892^\circ \text{ F.}$  as applying to that aluminum alloy and  $1070^\circ \text{ F.}$  as applying to the high nickel cast iron of band 10, then

$$u_{Al\ 142} = 2.187 \times 14.9 \times 10^{-6} \times 892 \quad (1)$$

$$= .029''$$

$$u_{Ni} = 2.187 \times 10.7 \times 10^{-6} \times (1140^\circ - 70) \quad (2)$$

$$= .025''$$

$$u_{Al\ 142} - u_{Ni} = .004'' \quad (3)$$

<sup>1</sup> Solidification temperature of #142 Alloy.

This shows that if the composite structure is to remain intact, then a force must be imposed on the insert 10 at the bond 13 which is great enough to cause a radial distortion inward of  $.004''$ . In order to obtain this factor, the principles of hydrostatic pressure are employed as applicable here because the conditions are the same, considering that the freezing aluminum alloy is essentially a liquid. It follows that

$$u = \frac{r_0 p_0}{E} \left( \frac{r_0^2 + r_i^2}{r_0^2 - r_i^2} - \mu \right)$$

where

$u$ =radial distortion produced by

$p_0$ =unit force in pounds per square inch

$E_{Ni}$ =Young's Modulus= $16 \times 10^6$

$r_0$ =outer radius= $2.750''$

$r_i$ =inner radius= $2.187''$

$\mu$ =Poisson's ratio=.256, as these factors are defined at page 241, "Strength of Materials" by Stephen P. Timoshenko, second edition, 1941, vol. II, D. Van Nostrand, New York.

Transforming the foregoing equation to solve for  $p_0$

$$\begin{aligned} p_0 &= \frac{u E}{r_0 \left( \frac{r_0^2 + r_i^2}{r_0^2 - r_i^2} - \mu \right)} \\ &= \frac{(.004) (16 \times 10^6)}{2.75 (2.750^2 + 2.187^2) - (2.750^2 - 2.187^2) (.256)} \\ &= \frac{6.4 \times 10^4}{2.75 \times 4.184} = 5600 \text{ lb./in.}^2 \end{aligned} \quad (4)$$

Considering the inner surface of an inserted ring band 10 to be  $1''$  long axially, the strength contribution of the bond at 13 is at least 9,000 pounds, and the two lateral edges of the band are stressed in shear. With an end area for a  $1''$  band of  $.563 \times 1.000 \times 2 = 1.13$  sq. in., and assuming a reasonable shear value of 6,000 pounds per square inch, the unit force will be  $6,000 \times 1.13 = 6800$  pounds, or a total of all forces of 15,800 pounds contributed solely by the bond at 13 and neglecting the shrink pressure on the sides of the insert which is negligible. This analysis accordingly shows that the bond at 13 between the insert 10 and the aluminum body of a piston is adequate to withstand the stresses of use, and many hours of use of the pistons of this invention demonstrate that the computation

is conservative, as there have been no failures of such pistons.

Although it has been suggested heretofore that high expanding ring bands be used, although without use of the essential bond heretofore described, applicant also has found that gray cast iron of low modulus of elasticity can be used as ring band material with beneficial results providing that gray iron of a modulus below  $16 \times 10^6$  is selected, preferably between  $11 \times 10^6$  and  $15 \times 10^6$ . Assuming the same conditions as before with Alcoa Al32 alloy as the piston body material and a low modulus gray cast iron as the band material, then adapting Formulae 1, 2 and 3 as 1', 2' and 3', it follows that

$$u_{Al\ Al32} = 2.187 \times 892 \times 12.3 \times 10^{-6} \quad (1')$$

$$= .024''$$

$$u_{c. 1.} = 2.187 \times 1015 \times 7.8 \times 10^{-6} \quad (2')$$

$$= .017''$$

$$u_{Al} - u_{c. 1.} = .007'' \quad (3')$$

Substituting in Formula 4 and changing values as indicated:

$$p_0 = \frac{(.007)(13.5 \times 10^{-6})}{2.75 \times 4.184} \quad (4')$$

$$= 8200 \text{ lbs./in.}^2$$

or a stress condition only 30% more than the case of high nickel cast iron and Alcoa 142 alloy which has withstood many hours of rigorous engine testing.

When the use of low modulus gray iron with Alcoa 142 alloy is considered, an artificially-produced distortion of .029-.017 or .012 is produced in the aluminum alloy. Substituting this value for .007 in Formula 4' gives an indication of stresses of the order of 14,000 pounds per square inch unit force, which considering the conservatism of the computation, serves amply to explain why such pistons showed no sign of failure in an engine after over 500 hours of rigorous usage.

The foregoing computations are based on the assumption that for relatively short axial lengths of insert 10, axial stresses can be neglected. However, where the axial length of an insert like 10 is materially greater than the 1 inch length assumed above, the axial stress is a very considerable part of the whole stress and, therefore, cannot be neglected. However, the strength of the bond at 13 of the piston of this invention provides a large factor of safety and hence, the band 10 may be safely widened axially to accommodate the next adjacent groove 12', if desired, although the upper one or two rings usually suffer the greatest wear and hence, need the iron band support more than lower rings.

Although a preferred embodiment of the bimetallic piston of this invention has been illustrated and described herein, it is to be understood that the invention is not limited thereby, but is susceptible of changes in form and detail within the scope of the appended claims.

I claim:

1. A piston for an internal combustion engine, comprising a cylindrical body portion formed of a light metal of relatively low strength, a band of a high strength ferrous metal encircling said body portion and embedded therein, and a film of an alloy of the body portion metal and the ferrous metal of the band interposed between the body and the abutting band surfaces for bonding them together.

2. A piston for an internal combustion engine, comprising a cylindrical body portion formed

of a light metal of relatively low strength of the class consisting of aluminum and aluminum base alloys, a band of a high strength ferrous metal encircling said body portion and embedded therein, and a film of ferro-aluminum alloy interposed between the body and the abutting band surfaces for bonding them together.

3. A piston for an internal combustion engine, comprising a cylindrical body portion formed of a light metal of relatively low strength, a band of a high strength ferrous metal having a modulus of elasticity below  $16 \times 10^6$  and encircling said body portion and embedded therein, and a film of an alloy of the body portion metal and the ferrous metal of the band interposed between the body and the abutting band surfaces for bonding them together.

4. A piston for an internal combustion engine, comprising a cylindrical body portion formed of a light metal of relatively low strength, a band of a high strength ferrous metal having a modulus of elasticity of between about  $11 \times 10^6$  and about  $15 \times 10^6$  and encircling said body portion and embedded therein, and a film of an alloy of the body portion metal and the ferrous metal of the band interposed between the body and the abutting band surfaces for bonding them together.

5. A piston for an internal combustion engine, comprising a cylindrical body portion formed of a light metal of relatively low strength, a band of low modulus cast gray iron encircling said body portion and embedded therein, and a film of an alloy of the body portion metal and the ferrous metal of the band interposed between the body and the abutting band surfaces for bonding them together.

6. A piston for an internal combustion engine, comprising a cylindrical body portion formed of a light metal of relatively low strength, a band of cast iron having a modulus of elasticity below  $16 \times 10^6$  and encircling said body portion and embedded therein, and a film of an alloy of the body portion metal and the ferrous metal of the band interposed between the body and the abutting band surfaces for bonding them together.

7. A piston for an internal combustion engine, comprising a cylindrical body portion formed of a light metal of relatively low strength, a band of cast iron having a modulus of elasticity between about  $11 \times 10^6$  and  $15 \times 10^6$  and encircling said body portion and embedded therein, and a film of an alloy of the body portion metal and the ferrous metal of the band interposed between the body and the abutting band surfaces for bonding them together.

8. A piston for an internal combustion engine, comprising a cylindrical body portion formed of a light metal of relatively low strength of the class consisting of aluminum and aluminum base alloys, a band of a high strength ferrous metal having a modulus of elasticity of between about  $11 \times 10^6$  and about  $15 \times 10^6$  and encircling said body portion and embedded therein, and a film of ferro-aluminum alloy interposed between the body and the abutting band surfaces for bonding them together.

9. A piston for an internal combustion engine, comprising a cylindrical body portion formed of a light metal of relatively low strength of the class consisting of aluminum and aluminum base alloys, a band of low modulus cast gray iron encircling said body portion and embedded therein, and a film of ferro-aluminum alloy inter-

posed between the body and the abutting band surfaces for bonding them together.

10. A piston for an internal combustion engine, comprising a cylindrical body portion formed of a light metal of relatively low strength of the class consisting of aluminum and aluminum base alloys, a band of cast iron having a modulus of elasticity between about  $11 \times 10^6$  and  $15 \times 10^6$  and encircling said body portion and embedded therein, and a film of ferro-aluminum alloy interposed between the body and the abutting band surfaces for bonding them together.

CHARLES E. STEVENS, JR.

REFERENCES CITED

The following references are of record in the file of this patent:

UNITED STATES PATENTS

| Number       | Name              | Date          |
|--------------|-------------------|---------------|
| 1,807,689    | Deputy            | June 2, 1931  |
| 1,946,081    | Koch              | Feb. 6, 1934  |
| 5 1,979,335  | Mahle             | Nov. 6, 1934  |
| 2,123,181    | Deputy            | July 12, 1938 |
| 2,255,006    | Graham            | Sept. 2, 1941 |
| 2,265,243    | McCullough et al. | Dec. 9, 1941  |
| 10 2,278,958 | White et al.      | Apr. 7, 1942  |
| 2,285,811    | Gay               | June 9, 1942  |
| 2,328,788    | Deputy            | Sept. 7, 1943 |

FOREIGN PATENTS

| Number     | Country       | Date          |
|------------|---------------|---------------|
| 15 581,527 | Great Britain | Oct. 16, 1946 |
| 566,312    | France        | Nov. 20, 1923 |